

July 8, 1958

J. S. NACHTMAN ET AL

2,842,440

PROCESS OF MAKING STRUCTURAL MATERIAL BY HEAT  
BONDING WIRE FILAMENTS  
Filed Dec. 18, 1953



INVENTORS  
JOHN S. NACHTMAN  
BY JOHAN BJORKSTEN  
*John S. Nachtmann*  
Attorney

## PROCESS OF MAKING STRUCTURAL MATERIAL BY HEAT BONDING WIRE FILAMENTS

John Simon Nachtman, Washington, D. C., and  
Johan Bjorksten, Madison, Wis.

Application December 18, 1953, Serial No. 399,085

7 Claims. (Cl. 75—208)

This invention relates to making a structural material by laminating metallic filaments provided with essentially metallic coatings and to shaped bodies made in this way.

It is well known that molecular orientation of a material such as a metal is often produced by drawing such material into the form of fine filaments. Fine filaments of such a material exhibit remarkably high tensile strength. The possibilities of providing a structural material of extremely high tensile strength by utilizing filaments of this type provided with metallic coatings have not heretofore been fully realized.

It is therefore an object of this invention to provide a method for making structural material of extremely high tensile strength by utilizing metallically coated metallic filaments.

Another object is a method for making a shaped metallic body by laminating together fine metallic filaments provided with coatings of metal or metal oxide.

Another object is a shaped body of structural material formed in this manner.

Further objects will become apparent from the drawing and the following detailed description in which it is our intention to illustrate the applicability of the invention without thereby limiting its scope to less than that of all those equivalents which will be apparent to those skilled in the art.

The drawing is a cross-sectional schematic view showing the preparation of coated metallic filaments suitable for the invention.

In accordance with a preferred embodiment of our invention we coat a steel rod 1 with copper coating 2 by electroplating and draw the resultant coated rod through a die 4 to reduce its diameter to from .020 to .0005 inch. A layer of generally parallel coated filaments prepared in this manner or prepared by coating previously drawn filaments is placed between suitably shaped platens or dies and the copper coatings are combined into a continuous media of copper surrounding the steel filaments by heating the structure or by heating the structure and at the same time exerting pressure thereon or by exerting pressure thereon without substantial heating. The optimum temperature is in any event below the melting point of the coating metal for heavy coatings, but at any temperature, even above the melting point, for thin coatings.

Instead of providing the metallically coated metal filament by drawing a coated rod through a die we may also suitably coat a fine metal filament after it is drawn.

In accordance with our invention we may use any one or more of the following metals or alloys thereof as materials from which to make the filaments:

|                 |            |
|-----------------|------------|
| Steel           | Bronze     |
| Stainless steel | Tin        |
| Chrome steel    | Cobalt     |
| Monel           | Zirconium  |
| Nickel          | Aluminum   |
| Copper          | Molybdenum |

Other metals, melting preferably above 900° F., and adapted to provide strong filaments.

The coating 2 which may be placed on the rod prior to drawing or placed on the filament after drawing may suitably comprise one or more of the above metals or alloy thereof or one or more of the following metals or alloy thereof:

|          |        |
|----------|--------|
| Antimony | Indium |
| Bismuth  | Zinc   |
| Cadmium  | Lead   |

10 The metals herewith stated as being suitable for coating metals may also be utilized in alloys suitable for providing filaments. Similarly metals listed above as particularly suitable for providing filaments may be utilized in alloys suitable for coatings. The coating may also comprise an oxide of a metal or an oxidation product of a metal alloy.

The coating need not consist of only one metal, metal alloy thereof or oxide; the rod or filament may be coated first with one metal or alloy thereof, then may be additionally coated with another metal or alloy thereof, then may be coated additionally with another metal or alloy thereof. The rod (prior to drawing) or filament (after drawing) thus coated may be heated to cause diffusion of the metals of the several coatings into one another or to cause diffusion of the coating next to the rod or filament into the rod or filament itself, or both.

The coating may be applied by any one of the methods known to the art. The metal coating may be applied by gas-plating, e. g. by passing a hot metal rod or

30 filament through a gaseous metallic compound such as a metallic carbonyl, formate, hydride, or the like, adapted to decompose upon contact with the hot rod or filament and to deposit thereon the metal of the aforesaid metal compound as a decomposition product. A metal coating may be deposited by electroplating. A coating may be deposited by evaporation of the coating material in a vacuum, also referred to as vacuum-sputtering or vacuum spattering. The rod or filament to be coated may be passed through a molten bath of the coating metal. A

40 metal may also be coated onto the rod or filament by passing through a bath of a light hydrocarbon vehicle having suspended therein particles of the coating metal and then passing the rod or filament through a furnace to cause the hydrocarbon vehicle to evaporate and to cause the particles of coating metal deposited thereon to coalesce into a continuous coating. The metal, or alloy thereof, or oxide thereof, may be coated by dipping a rod or filament in a solution or suspension of a compound of the material to be deposited thereon. The article thus coated with solution may be removed from the bath and heated to cause decomposition of the compound and deposition of the material to be coated.

45 As shown in the figure, heat 3 is applied to rod 1 provided with coating 2 which is continuously drawn through a die 4 to provide coated filament 5.

The rod before or after coating may be heat-treated in any suitable, if desired, to provide improved properties for subsequent processes such as may result from such heat-treating. The coated filament 5 after being drawn may also be heat-treated to provide desired properties but heat-treating of such filaments must be carried out with extreme care to avoid deleterious effects on the high tensile strength of the filament resulting from its orientation during drawing.

50 65 The process may be carried out in accordance with any one of the following patents: 2,490,700, 2,402,834, 2,428,318, 2,428,033 and 2,637,896 in order to provide, for example, a bronze coating by causing a tin coating and a copper coating to diffuse into one another; in order to provide a stainless steel coating by causing layers of copper, nickel and steel to diffuse into one another; or

to provide a Monel coating by causing layers of nickel and copper to diffuse into one another.

In accordance with the invention, laminates are made from the coated filaments prepared as described above. Such laminates consist of the filaments bonded together with the material of the coating thereon by diffusion of the coating material on each filament into the coating material on adjacent filaments. Laminates are formed by placing a suitably large bundle of coated fibers between platens or shaped dies of a press or rolls of a rolling mill without the addition of a metal or metallic compound or any other compound as a binder material. Sufficient pressure is exerted by the platens or dies or rolls to force the bundle into a compact mass. Bonding may then be caused to occur by applying heat or pressure (as in cold rolling) or both heat and pressure. Generally the application of both heat and pressure is preferred, the heat being sufficient to cause bonding by diffusion without heating the filament material to a temperature which would be deleterious to the physical properties of the filaments.

The terms "continuous medium," "continuous media," "continuous bonding medium" and "continuous bonding agent" are used throughout to refer to material which extends throughout an article or shaped body in such a manner that a theoretical point contained within the interior of the bonding material may travel from any point on any surface of the article to any other point on any other surface without passing outside of said housing material or passing through any interface between said bonding material and any other material.

The invention is further illustrated by the following examples:

*Example 1*

A rod  $\frac{1}{4}$  inch in diameter and 6 feet long of SAE 1066 steel is placed in a copper electroplating bath and copper is electroplated thereon until the plating has reached a thickness of approximately .020 inch. The coated rod is then heated, one end is swaged and passed into a die as shown in the illustration and the coated rod is drawn down to a coated filament having an approximate outside diameter of .002 inch, the filament having a very thin coating of copper.

Such filaments are placed between platens of a press; heat and pressure are exerted thereon to provide a flat structural article of a high tensile strength, comprising a continuous medium of copper having steel filaments disposed therethrough.

*Example 2*

Filaments prepared in accordance with Example 1 are immersed in an electroplating bath; nickel is plated thereon. The resultant copper coated filaments having a nickel outer coating are heated to cause slight diffusion of the nickel coating into the copper coating; layers of such filaments in somewhat parallel relationship are placed between matched metal dies in a press so that each filament extends at least from one side of the mold cavity to the other side and heated while being maintained under pressure to provide a shaped article of great strength, with a continuous medium of nickel as bonding agent.

*Example 3*

A bundle of filaments prepared as in Example 1 are placed between shaped ceramic dies so that all filaments extend beyond the die cavity at each end and heated at below the melting point of the copper coating while being maintained under contact pressure to provide a structural article comprising steel filaments bonded together with a substantially continuous medium of copper, having great strength.

Laminates prepared in accordance with the invention may be heat-treated to improve their properties but care

must be exercised to avoid undesired loss of properties in the fine filaments.

*Example 4*

5 A rod  $\frac{3}{8}$  inch in diameter of AISI C1141 steel is coated with a .026 inch coating of nickel by electroplating. The rod thus nickel coated is drawn down to a diameter of .125 inches and then swaged and then passed through 10 progressive dies while still above the softening temperature until .020 inch in diameter. At the output end of the .020" diameter die it is heated and then by drawing at high speed drawn down to .005 to .010" diameter.

The extremely fine filaments prepared in this manner are provided with an additional coating of nickel by gas- 15 plating from nickel carbonyl and are then placed between shaped polished matched steel dies in a press and subjected to a pressure of approximately 90,000 pounds per square inch, which is maintained for approximately one hour while the dies are maintained at a temperature 20 below the melting point of the nickel and the steel, sufficiently low to avoid deleterious effect on the tensile strength of the steel filaments resulting from their orientation during drawing. The steel filaments are thus bonded with a continuous medium of nickel.

*Example 5*

Copper wire .0035 inch in diameter is passed through a bath of molten lead. A thick plate is formed by pressing a bundle of such coated wires between matched metal 30 dies at approximately 50,000 pounds per square inch.

*Example 6*

Steel music wire (SAE 1085 steel) .007 inch in diameter 35 is coated by passing it through a molten bath of zinc-aluminum alloy sold commercially as Zamac 3. A bundle of wire thus coated is placed between dies in a press so that each filament extends beyond the die cavity and a valve housing is made by pressing at 900 pounds per square inch and heating to the melting point of said 40 alloy to cause the coatings to diffuse into one another.

*Example 7*

A nickel rod (melting at approximately 2646° F.) 45 having a diameter of approximately .005 inch is provided with a coating of silicon bronze by casting around the rod a molten alloy having the composition:

|           | Percent |
|-----------|---------|
| Copper    | 95.8    |
| Manganese | 1.1     |
| Silicon   | 3.1     |

The coated rod is drawn through a series of dies to 55 reduce its diameter to .002 inch. Layers of the resulting coated filaments are placed between the platens of a press and subjected to heat and pressure to form a reinforced structural plate of high tensile strength.

*Example 8*

A tungsten wire .005 inch in diameter is coated with 60 an aluminum bronze by drawing it at a sharp angle over a series of ten blocks of an alloy having the composition:

|          | Percent |
|----------|---------|
| Copper   | 91.0    |
| Aluminum | 7.0     |
| Silicon  | 2.0     |

The blocks of hard bronze alloy have a tensile strength of 65 88,000 p. s. i. and a melting point of 1930° F. The 70 harder tungsten wire removes the softer bronze by abrasion and the abraded particles cling to the wire. The particles are caused to coalesce into a continuous coating by passing the wire through an oven maintained at a temperature of about 1950° F.

75 A mass of the thus-coated filaments are placed between

matched metal dies in a press and an aircraft component is made by applying heat and pressure.

*Example 9*

Steel filaments .001 inch in diameter are coated with a tin coating .000055 inch thick by electroplating. Layers of thus-coated filaments are placed between the platens of a press in such manner that the filaments in each layer are parallel to one another and filaments in one layer are at an angle to the filaments in the next adjacent layer. The filaments are subjected to heat and pressure and the tin is thus caused by diffusion to provide a continuous bonding media. In this manner is formed a plate containing steel filaments extending from one part of the plate to the other in layers, the filaments in each layer being parallel and the layers being parallel to one another, bonded together with a continuous bonding media of tin.

It may be seen that in each of the examples, the article made according to the invention is porous if thin coatings are provided on the filaments and is non-porous if relatively thick coatings are provided on the filaments. Only the coating material is provided as material adapted to fill the interstices between the filaments of higher melting metal. No additional bonding agent is provided as would be the case if molten metal were cast on the filaments. Thus by controlling the thickness of coating we may control the size of the interstices and thus adjust the properties which we wish to obtain. By providing relatively large interstices we may provide a material which has great strength while being relatively light. On the other hand for some applications we may wish to provide a material which is particularly resistant to passage of liquids or gases therethrough and in this event we would generally provide filaments with relatively thick coatings so that upon being subjected to high pressure and to a temperature adapted to cause diffusion of the coating material, the material of the coatings will flow together and fill the interstices.

*Example 10*

A single layer of parallel strands of tin-coated copper wire is cold-rolled to provide a flat sheet and immediately heat-treated to provide a bonded flat sheet by diffusion of the tin at the adjacent surfaces.

*Example 11*

Two layers of bronze-coated nickel wire are heated and passed between a pair of hot rolls while being maintained in the form of two layers of parallel wires, the wires in one of the two layers being at an angle to those in the other layer. A flat article comprising flattened wires bonded together by partial diffusion of the coating on each wire into the coating of the adjacent wires, is thus formed. The article thus comprises filaments of nickel extending from one side of the article to the other bonded with a continuous media of copper.

*Example 12*

A steel filament is provided with a copper coating and then with a nickel coating by electroplating and is then heat-treated to cause the nickel coating and copper coating to partially diffuse into one another. A plurality of the thus-coated filaments are placed with any particularly desired orientation, with a large number of the filaments parallel to one another, between the dies of a press adapted to provide an article such as a gear housing. The press is then closed and the structure is maintained at a temperature adapted to provide for substantially complete diffusion of the materials of the two coatings into one another and for a time sufficient to provide for partial diffusion of the coating of each filament into the coating of each adjacent filament, to thereby bond the filaments together.

The article is then removed and as thus prepared com-

prises filaments bonded with a continuous media of non-homogeneous or homogeneous alloy of nickel and copper.

It may thus be seen that our invention relates to shaped bodies, structural shapes or the like comprising filaments which extend from one side of the body to the other side of the body.

Our invention further relates to such articles in which bonding between the filaments is provided by a continuous media of metal or metal oxide.

10 Our invention further relates to such bodies or articles wherein bonding is accomplished by diffusion of the coating material of each filament into coating material of adjacent filaments.

15 Our invention further relates to such articles or bodies wherein bonding is provided entirely by coating provided on the filaments, without the addition of any additional material such as might be provided by casting molten metal around the filaments or adding solder or eutectic welding alloy or the like in the form of wire or rods or the like.

Metal oxides may be utilized to provide insulating properties.

It may thus be seen that the invention is broad in scope and is not to be limited excepting by the claims.

25 Having thus disclosed our invention, we claim:

1. The process of providing a shaped body comprising metal wire filaments extending therethrough which comprises the steps of providing a plurality of metal wire filaments .001" to .010" in diameter coated with at least 30 two layers .00001" to .001" thick each of said layers being a non-powdered continuous substantially homogeneous substance selected from the group consisting of metals and oxides thereof of different composition than said filament, compacting a group of said filaments under 35 pressure sufficiently low to prevent elongation and cross-sectional deformation of said filaments and while maintaining such pressure thereon, applying heat to said compacted mass at a gradually increasing rate to alloy said layers with each other to thereby join said filaments together, said heat being applied at a rate which prevents the temperature of said compacted mass from exceeding the melting point of any component thereof.

2. The process of claim 1 characterized by causing said filaments to be oriented parallel to one another prior to being compacted.

3. The process of claim 1 characterized by causing a portion of said filaments in said group to be parallel to one another and another portion of said group of filaments to be parallel to one another but to be at an angle to the filaments in said first portion.

4. The process of claim 1 further characterized by providing said group of filaments by first laying a group of coated filaments parallel to one another in a bottom mold half and then laying a second group of filaments 55 parallel to one another but at an angle to said first group of filaments on top of said first group, and by then compacting the resultant assembly of such coated filaments by forcing a top mold half against said bottom mold half.

5. The process of claim 1 further characterized by 60 commencing said heating with said compacted filaments at a temperature below 200° F. and then heating said filaments over a period of at least one half hour to a temperature above 800° F. and below the transition temperature of the metal of the filaments.

6. The process of providing a shaped body comprising 65 metal wire filaments extending therethrough which comprises the steps of providing a plurality of ferrous alloy wire filaments .001" to .010" in diameter coated with at least two layers .00001" to .001" thick, each of said layers being a non-powdered continuous substantially homogeneous substance selected from the group consisting of metals and oxides thereof of different composition than said filament, then compacting a group of said filaments under pressure sufficiently low to prevent elongation and cross-sectional deformation of said filaments and while

maintaining such pressure thereon, applying heat to said compacted mass at a gradually increasing rate to alloy said layers with each other to thereby join said filaments together, said heat being applied which prevents the temperature of said compacted mass from exceeding the melting point of any component thereof, further characterized by commencing said heating with said compacted filaments at a temperature below 200° F., and then heating said filaments over a period of at least one half hour to a temperature above 800° F. and below the 10 transition temperature of the metal of said filaments.

7. The process of providing a shaped body comprising metal wire filaments extending therethrough which comprises the steps of providing a plurality of metal wire filaments .001" to .010" in diameter coated with at least one layer .00001" to .001" thick, said layer being a non-powdered continuous substantially homogeneous substance selected from the group consisting of metals and oxides thereof of different composition than said filament, compacting a group of said filaments under pressure sufficiently low to prevent elongation and cross-sectional deformation of said filaments and while main-

5 taining such pressure thereon, applying heat to said compacted mass at a gradually increasing rate to alloy said layers in adjacent filaments with each other to thereby join said filaments together, said heat being applied at a rate which prevents the temperature of said compacted mass from exceeding the melting point of any component thereof.

## References Cited in the file of this patent

## UNITED STATES PATENTS

|           |               |               |
|-----------|---------------|---------------|
| 867,659   | Hoopes        | Oct. 8, 1907  |
| 1,292,659 | Speed         | Jan. 28, 1919 |
| 1,336,449 | Trunk         | Apr. 13, 1920 |
| 1,704,256 | Lorenz        | Mar. 5, 1929  |
| 1,708,193 | Sherwood      | Apr. 9, 1929  |
| 1,919,730 | Koenig et al. | July 25, 1933 |
| 2,030,229 | Schwarzkopf   | Feb. 11, 1936 |
| 2,146,823 | Karmazin      | Feb. 14, 1939 |
| 2,219,434 | White         | Oct. 29, 1940 |
| 2,273,589 | Olt           | Feb. 17, 1942 |
| 2,499,977 | Scott         | Mar. 7, 1950  |